

## UNITED STATES PATENT OFFICE.

THOMAS A. MOORMANN, OF MILWAUKEE, WISCONSIN, ASSIGNOR TO KINITE CORPORATION, OF MILWAUKEE, WISCONSIN, A CORPORATION OF WISCONSIN.

## STEEL ALLOY AND PROCESS OF MAKING THE SAME.

No Drawing.

Application filed November 11, 1926. Serial No. 147,852.

My invention relates to a steel alloy and process of making the same, and refers particularly to the making of alloy steel castings.

5 In the ordinary well-known practice of making steel castings, a strongly tenacious film of oxide forms on the surface of the molten metal when the correct pouring temperature is reached. This film not only is 10 present on the surface of the molten metal in the pouring ladle, but is also found on the surface of the metal after it has been cast in the mold.

15 In the process of pouring, this film carries with it entrained sand and other extraneous matter, which results in imperfections in the surface of the casting. In order to remove these surface defects, excessive machining of the casting is necessary.

20 The above difficulties of making good castings are encountered particularly in the case of alloy steels which contain chromium and other similar alloying elements.

It is one of the objects of my invention 25 to so treat the steel that the film of oxide forming on the surface of the molten metal and causing surface defects in the casting, is substantially eliminated, with the result that the amount of machining necessary to 30 give the casting a perfect finish is very largely decreased.

I have found that this result may be accomplished by the use of the addition of a 35 relatively small quantity of boron, which, particularly in the case of alloys in which chromium is used, forms a very fluid flux, which is without deleterious effect on the surface of the casting.

I have also found that a further advantage resulting from the use of boron is that the size of the risers can be greatly reduced 40 in obtaining solid castings, the effect of the boron being to lower the temperature at which the steel becomes completely solid so 45 that the risers can be kept in a molten condition for a longer time, thus allowing the addition of molten metal as the level of the molten metal in the risers sinks—a condition which is normally brought about as the 50 metal solidifies in the casting proper.

A further object of my invention is to provide an alloy having the desirable surface features pointed out above, and which,

particularly when heat treated, will present great resistance to wear and abrasion. 5

The various objects of my invention are accomplished in the manner which I shall now describe.

The steel is preferably made in an acid electric furnace, the desired alloying elements being preferably added in the form of ferro alloys to give required analysis of the finished material. 60

Shortly before the tapping of the furnace, I add to the charge boron, either in 65 the form of ferro-boron, or other suitable alloy, such as boron manganese. I have found that approximately .40 per cent boron figured on the entire furnace charge gives 70 satisfactory results, although the amount of boron added to the charge may vary between .20 and 2.6 per cent without departing from the spirit of my invention. Particularly in 75 the presence of chromium, a large part of the boron goes into the slag, forming a very fluid slag. At the same time, it serves to eliminate from the metal impurities, such as entrained oxides. The boron contained in the finished steel is ordinarily found to 80 be between .05 and .20.

Although I have described the use of boron particularly as a furnace addition, the boron in the form of ferro-boron, or other suitable alloy, may, if desired, be added in the ladle. If this is done, sufficient time 85 should be allowed for the uniform alloying of a portion of the boron with the steel, and the metal should, of course, be allowed to cool to the proper pouring temperature 90 before pouring.

In order to cause a thorough mixture of the boron with the steel, I prefer to stir the molten metal either in the furnace or in the ladle.

I have found that a typical analysis of the 95 alloy in connection with which my improved process may be advantageously used, is as follows:

|                                    | Per cent. |
|------------------------------------|-----------|
| Carbon                             | 1.50      |
| Chromium                           | 13        |
| Cobalt                             | .70       |
| Molybdenum                         | 1.10      |
| Manganese                          | .80       |
| Silicon                            | .50       |
| Phosphorus and sulphur, each below | .02       |

In the finished casting, there would also be found from about .05 to about .20 per cent boron, as previously pointed out, although in some cases this amount may be advantageously increased up to approximately one per cent.

Considerable variations may be made from the typical analysis which I have given without departing from the spirit of my invention. For example, carbon may be between 1.2 and 3.5 per cent; chromium between 8 and 20 per cent. In place of cobalt and molybdenum, as given in the typical analysis above mentioned, I may use tungsten, uranium, zirconium or titanium, either with or without cobalt or molybdenum, or both, the combined percentage of the elements cobalt, molybdenum, tungsten, uranium, zirconium and titanium being approximately between 20 one and two per cent.

Castings which are made of the alloy which I have described are very hard and practically unmachinable, but upon annealing may be readily machined. It has been found that these castings may be heat treated or annealed without distortion and are practically immune from danger of cracking. Rockwell hardness values C-63 are obtainable by air cooling without quenching 30 or use of a cooling blast.

The physical properties of the heat treated castings are tensile strength about 125,000 pounds per square inch, and compressive strength about 420,000 pounds per square 35 inch.

The heat treated castings made according

to my invention have high resistance to abrasion and are particularly adapted for use as tools, such as forming dies, and the like.

It has been found that the hardness and resistance to abrasion extends through the entire mass of the heat treated castings and is not confined to the surface thereof—a feature which is most valuable and desirable in connection with tools such as dies, which 45 are frequently redressed.

The steel may also be heat treated so that it will be left in the austenitic condition, and therefore non-magnetic.

It is also possible to forge steel made in accordance with my invention; and in the hardened condition, I have found that such forgings have a tensile strength of approximately 220,000 pounds per square inch.

I have also found that a steel made in accordance with my invention does not have its hardness altered or impaired by subjecting the hardened steel to temperatures up to 1100 degrees Fahrenheit.

It will be apparent to those skilled in the art that many changes could be made in the details of the invention which I have described without departing from the spirit or scope of my invention.

I claim:

A steel alloy of substantially the following composition: approximately carbon 1.50%, chromium 13%, cobalt .70%, molybdenum 1.10%, boron .05 to .20%.

Signed at Milwaukee, Wisconsin, this 1st 70 day of November, 1926.

THOMAS A. MOORMANN.